

May 28, 1935.

E. B. McCONNELL

2,002,670

PROCESS OF MAKING ASPHALT

Original Filed July 3, 1931



INVENTOR.

Elliott B. McConnell

BY

Gray, O'Brien & Gray  
ATTORNEYS.

## UNITED STATES PATENT OFFICE

2,002,670

## PROCESS OF MAKING ASPHALT

Elliott B. McConnell, Cleveland, Ohio, assignor  
to The Standard Oil Company, Cleveland,  
Ohio, a corporation of Ohio

Original application July 3, 1931, Serial No.  
548,601. Divided and this application June 30,  
1934, Serial No. 733,252

2 Claims. (Cl. 196—74)

A fundamental difficulty in the manufacture of asphalt has centered about the limitation of oxidizing action. In the customary procedure in which petroleum has been distilled, with removal of progressively heavier cuts down to lubricating fractions, and the bottoms or residuum has then been subjected to the action of air as bubbled through a perforated pipe along the bottom of the still, the amount of exposure and contact action has been so limited as to necessitate very prolonged treatment, two or three days for a batch; and besides the draw-back of such a large time factor there is the further difficulty that such prolonged subjection of hydrocarbons to the high temperatures necessary, effects detrimental decomposition tending to erratic and deficient results. In accordance with the present invention however, it now becomes possible to subject asphalt-forming residuum to a thorough-going oxidation treatment with relatively small time requirement, and besides a continuous type procedure, as opposed to batch-wise, is available.

To the accomplishment of the foregoing and related ends, the invention, then, comprises the features hereinafter fully described, and particularly pointed out in the claims, the following description and the annexed drawing setting forth in detail certain illustrative embodiments of the invention, these being indicative however, of but a few of the various ways in which the principle of the invention may be employed.

In said annexed drawing:—

The sole figure is a semi-diagrammatic sectional elevation showing apparatus contemplated.

A petroleum residuum, as obtained for instance by distilling petroleum and removing the naphtha and progressively heavier cuts on through the lubrication fractions, for example the residuum or bottoms from the distillation of Mid-Continent petroleum as reduced to about 7-8 per cent is, in molten or adequately fluidified form, projected in finely divided spray or atomized condition counter-currently to a supply of air. For such fine division, finely perforated or porous plates or air-atomizer heads may be employed, especially heads in which the subdivision of liquid is effected by the pressure applied and the emergence through passages affording a fine breaking up of the liquid body with formation of very small droplets or mist particles as projected into the air. In the form of equipment illustrated, an atomizer-spray head 2 is arranged at the top of a suitable chamber or tower 3, and is supplied by pipe 4 from a source of residuum,

for instance a pump 5 serving to provide a requisite distribution pressure. The spray-head 2 is a finely perforated diaphragm. On account of the difficulty in attaining a desirably fine perforation by direct mechanical punching, it is preferable to provide such perforated diaphragm in the form of a porous plate or plates making up a header of sufficient extent, and such plates may be of any suitably porous material, as for example aluminum oxide, porcelain or other ceramic material in which pores may be conveniently formed by proportioning the granular raw material from which the plates are initially molded. Various degrees of size of pore openings may be had in materials of this order. Desirably, a heating means, as for instance a steam coil 20, is provided adjacent the diaphragm 2, for facilitating melting out of residuum which may become solidified or frozen on occasion of temporary shut-down. At the bottom of the chamber 3 an air inlet is provided and this may conveniently take the form of a perforated pipe 6 connected with a blower or compressor 7, for supply of a body of air in the chamber. At the top an off-take pipe 8 may lead through a condenser 9 to a receiver 10, and if desired an eduction air pump to blower at the end of the vent pipe 11.

As above indicated, the residuum, for instance as coming from the final distillation zone, through pipe 12, and at a temperature of around 700° F., or lower, to about 400° F., is fed by the pump 5 to the atomizer head 2, where it is projected in finely divided atomized form, against a rising current of air introduced by pipe 6. As the finely divided residuum or mist-like particles leave the atomizer head, they are at once enveloped in an abundance of air, and with the elevated temperatures provided and the exaggerated surface exposure, oxidation proceeds effectively. The product collecting at the bottom of the tower may be drawn off through the pipe 13 to tanks, shipping drums, or whatever disposal is desired. In some cases, further treatment may be preferred by recycling the material through the pipe 14, the valves 15 and 16 being closed and the valves 17 and 18 being open. The pump 5 then recycles the material until a sample taken off at the sampling outlet 19, shows the desired specification characteristics. The effluent air proceeds through off-take pipe 8 and the condenser 9 to the discharge pipe 11, any condensable substances being collected in the receiver 10. Temperature control may be maintained as desired by the temperature of

the incoming residuum and the air. The air may be cooled in some cases as required, or it may be specially heated, or it may carry the heat acquired in the compressor.

5 Where it is desired to especially heat the air from the compressor, a heater 21 may be applied to the air pipe prior to its entrance into the tower, the heat being applied by any suitable means, such as furnace or a flue-gas connection.

10 This application is a division of my prior application Serial No. 548,601, filed July 3, 1931.

15 Other modes of applying the principle of the invention may be employed, change being made as regards the details described, provided the features stated in any of the following claims, or the equivalent of such, be employed.

I therefore particularly point out and distinctly claim as my invention:—

1. A process of making oxidized asphalt, which comprises forcing petroleum residuum through capillary diaphragm openings, projecting the finely divided residuum therefrom in counter-current flow, to air, and withdrawing the oxidized asphaltic product. 5

2. A process of making oxidized asphalt, which comprises forcing petroleum residuum through capillary ceramic openings, projecting the finely divided residuum therefrom in counter-current flow to air, and withdrawing the oxidized asphaltic product. 10

ELLIOTT B. McCONNELL. 15